

## UNITED STATES PATENT OFFICE

FRANK L. REMLEIN, OF NEW YORK, N. Y., ASSIGNOR TO E. I. DU PONT DE NEMOURS & COMPANY, OF WILMINGTON, DELAWARE, A CORPORATION OF DELAWARE

## PROCESS FOR VAT COLOR DYEING

No Drawing.

Application filed June 26, 1928. Serial No. 288,535.

This invention relates to a process of applying vat colors to materials and fabrics such, for example, as piece goods. More particularly it relates to an improved method of 5 developing the color on the goods.

The usual procedure in dyeing vat colors on piece goods is either to pad the cloth with reduced dyestuff and then develop in the jig, or to dye the piece goods in the padder and 10 then pass the goods through a second reducing solution containing caustic soda and hydrosulfite with or without the addition of color.

An object of my invention is a process of 15 vat color printing or dyeing in a single step. A further object of my invention is the development of the color by evaporation of the water remaining in the goods after padding.

I have found that after the dyeing is effected in the usual way by padding the cloth in a solution of reduced dyestuff, the color may then be developed by using the steam produced by the evaporation of the water remaining in the goods after they have passed 25 the pad rolls. The development may be effected by running the cloth over steam heated cans. It will be understood of course that other means of heating may be employed for this purpose. By the use of this method I 30 have found that extremely rapid production is possible and the dyeings produced are of the very best possible fastness obtainable with the particular dyestuff used.

This process may be used for dyeing with 35 vat colors in heavy as well as light shades.

By way of description of the process comprising my invention, the following illustrative example of dyeing on medium and light shades on light weight goods is given, but it 40 will be understood that other embodiments exist and may be practiced without departing from the spirit of my invention.

The goods to be dyed are passed into a padding solution comprising:

45 *For 160 gallons*

10 lbs. Ponsol blue GD double paste (color index Number 1113).

8 lbs. Du Pont hydrosulfite conc.

50 8 lbs. caustic soda.

8 lbs. animal glue.

1 lb. anthraquinone.

Reduce 10 min. at 130° F.

The goods are then passed through squeeze rolls and developed with steam by running 55 the wet goods directly on hot cans before the color is oxidized to its insoluble state.

As many apparently widely different embodiments of this invention may be made without departing from the spirit thereof, 60 it is to be understood that I do not intend to limit myself to the specific embodiments thereof except as indicated in the appended claims.

I claim:

1. In the process of vat color dyeing, the 65 steps which comprise padding the color in a solution of reduced dyestuff and developing the color with steam produced by evaporation of the water remaining in the goods after 70 padding.

2. In the process of vat color dyeing, the 75 steps which comprise padding the color in a solution of reduced dyestuff and developing the color by running the wet goods directly on hot cans before the color is oxidized to its insoluble state.

In testimony whereof, I affix my signature.

FRANK L. REMLEIN.

65

75

80

85

90

95